

# United States Patent Office

3,164,495

Patented Jan. 5, 1965

1

3,164,495

ULTRA HIGH STRENGTH ALLOY STEELS  
Clyde A. Furgason, Milwaukee, Wis., assignor to Ladish  
Co., Cudahy, Wis., a corporation of Wisconsin  
No Drawing. Filed Sept. 26, 1961, Ser. No. 140,674  
1 Claim. (Cl. 148—36)

This application is a continuation-in-part of my application Serial No. 82,969, filed January 16, 1961, now abandoned.

This invention relates to improvements in ultra high strength alloy steels and particularly to a steel that contains a minimum of strategic alloying elements while possessing high yield and ultimate strength when tempered at high temperatures and the ability to maintain high strength at elevated temperatures.

Users and manufacturers of hot work tool and die steels are constantly looking for improved steels which are stronger, tougher, have higher impact resistance, and can withstand higher temperatures. Most hot work die steels possess a secondary hardening characteristic which provides higher temperature resistance because high hot hardnesses can be obtained and retained when tempering at high temperatures. At the same time, these steels must be capable of being hardened deeply.

Prior to the present invention, the lowest alloy analysis which would impart secondary hardening was generally considered to be an alloy containing no less than 7% total alloying elements.

It is therefore an object of this invention to provide an alloy steel analysis containing only approximately 4% total alloying elements, that is deep hardening and possesses a secondary hardening characteristic plus good ductility. The alloy steel of this invention is applicable to critical hot work tool and die applications as well as to ultra high strength structural applications subject to elevated temperatures and both dynamic and static loading.

Aircraft, and more recently missile, manufacturers have been constantly seeking newer and better materials for utilization on critical parts where high strengths and strength/weight ratios could bring about substantial weight savings on the vehicles. Coupled with this trend toward lighter weight, higher strength is the increase in speed with an accompanying aerodynamic heating problem. This has necessitated high strength materials which are capable of withstanding sustained elevated temperatures without losing strength and ductility.

The abilities of aircraft and missile structural materials to perform under these conditions has necessitated a shift from the AISI 4340 type material and its modifications to the more highly alloyed materials (for example SAE H-11) (0.40% C, 5.0% Cr, 1.30% Mo, 0.50% V).

The reason for this shift is the need for a steel which can be heat treated to tensile strengths of 220,000 to 280,000 psi and retain sufficient toughness for landing gear, engine mounts, hot work tools and dies, and other structural applications. A greater problem was to provide an alloy steel capable of being heat treated to these high strengths and at the same time maintain its strength as aerodynamic heating increased the operating temperatures of the structures. The SAE H-11 type material possesses the combination of toughness at ultra high strengths and elevated temperature strength up to 900° F.—1000° F. It has a composition which produces secondary hardness which is essential for complete stress relief for maximum toughness. However, the SAE H-11 type material containing approximately 7% total alloy content is extremely sensitive to chemistry variations during tempering due to the fact that the tempering curve is very steep beyond the secondary hardening peak. The material is also susceptible to formation of carbide net-

2

works which adversely affect the heat treat response if cooling from the hot working temperature is not precisely controlled or executed properly. It has heretofore been generally believed that H-11 is the lowest alloy analysis that will impart secondary hardening.

It is therefore an object of the present invention to provide an improved alloy steel that possesses an extremely low alloying element content, thereby using a minimum of strategic materials, while possessing secondary hardening characteristics with good ductility especially at room temperature.

It is a further object of the invention to provide an alloy composition that possesses secondary hardening characteristics while only containing approximately 4% total alloy content, said alloy also possessing excellent high strength and toughness properties.

Many of the so-called ultra high strength steels rely on high Silicon contents to reduce temper brittleness while producing high strength levels when tempering between 400° F. and 700° F. It is therefore an object of the invention to provide an alloy steel which exhibits high strength with adequate ductility when tempered in excess of 1000° F., thereby providing maximum stress relief of quenching stresses as well as permitting distortion correction at high temperatures where correction is much simpler.

It is a further object of the invention to provide an alloy steel which restricts the amount of the alloying element silicon to less than 0.5%, thereby maintaining high stress rupture properties. Silicon contents in excess of 0.5% results in degradation of said stress rupture properties.

A still further object of the invention is to provide alloy steel which maintains higher elevated temperature stability than other secondary hardening alloys.

In the alloys of my prior patents Nos. 2,919,188, dated December 29, 1959, and 2,921,849, dated January 19, 1960, if it were attempted to heat treat to ultra high strength levels, the tempering temperature would have to be substantially lower than with the present invention as there would be considerably less relief of quenching stresses during tempering at the low temperature. The results of the present invention are obtained principally by substantially increasing the amount of molybdenum over that contained in the alloys of my prior patents, whereas to obtain the results of the present invention it would be conventional practice to substantially increase the amount of chrome to a level substantially affecting the cost of the alloy, as compared to the cost when molybdenum is moderately increased as in the present invention.

A further object of the invention is to provide an alloy steel which is suitable for use where superior toughness, wear resistance, elevated temperature strength, stress rupture strength and high impact load resistance are necessary, making it particularly suitable for elevated temperature structural, die and tool steel applications.

A further object of the invention is to provide an alloy steel which exhibits superior properties at room temperature when heat treated to a predetermined high tensile strength range, the alloy retaining high strength at elevated temperatures so that it can be used for applications where high strength at both room temperatures and elevated temperatures is required.

A further object is to provide an alloy steel which maintains a high yield to ultimate ratio at all strength levels up to 280,000 p.s.i.

A further object is to provide an alloy steel of low creep rate at elevated temperatures so that the material may be used where applications at high temperature stress are required for prolonged periods of time.

Other objects are to provide an alloy steel which exhibits less distortion in quenching, and which is weldable in heavy sections, while employing techniques and controls normally used in welding medium carbon low alloy materials with high hardenability.

It is a further object to provide an improved alloy steel that can, while in the fully heat treated condition be reheated several times to a temperature approaching 1000° F. without materially affecting the properties in order to facilitate straightening or correction of distortion due to quenching stresses or to accommodate cycles of heating and cooling encountered during normal operation.

In carrying out the invention, it has been discovered that a relatively high carbon range can be used in the

5 materials need be employed to obtain properties heretofore obtained by a much higher alloy content.

The following tables indicate the improved properties of the alloy steel of the present invention.

An average of the room temperature mechanical properties of the present alloy steel after normalizing at 1900° F., air quenching from 1850° F., and tempering as shown, are summarized in Table I. The maximum ultimate and yield strength with adequate ductility, as measured by the percent elongation and reduction of area, is achieved by tempering between 1000° F. and 1100° F. This temper produces an ultimate tensile strength of 265,000 to 275,000 p.s.i. a yield strength of 235,000 to 255,000 p.s.i. elongation of 9-10%, and a reduction of area of 35-45%.

TABLE I

Mechanical Properties at Room Temperature, Air Quenched From 1850° F. and Tempered as Shown

| Temper Temp., ° F. | U.S., p.s.i. | Y.S., p.s.i. | Percent Elong. in 2" | Percent Red. of Area | Rockwell "C" Hardness | Charpy V-Notch Impacts, ft. lbs. |
|--------------------|--------------|--------------|----------------------|----------------------|-----------------------|----------------------------------|
| 400                | 308,000      | 247,100      | 9.0                  | 26.8                 | 54                    | 14.2                             |
| 550                | 294,000      | 247,100      | 9.5                  | 34.1                 | 53                    |                                  |
| 700                | 274,000      | 231,600      | 9.5                  | 30.8                 | 52                    | 12.3                             |
| 800                | 270,200      | 232,900      | 10.5                 | 36.0                 | 52                    | 12.8                             |
| 850                | 268,000      | 232,000      | 12.0                 | 37.3                 | 52                    |                                  |
| 900                | 271,000      | 237,000      | 11.5                 | 38.9                 | 51                    | 14.3                             |
| 950                | 269,300      | 236,000      | 11.5                 | 35.7                 | 51                    |                                  |
| 1,000              | 277,200      | 248,900      | 12.0                 | 46.1                 | 53                    | 17.7                             |
| 1,050              | 277,500      | 255,600      | 11.0                 | 43.2                 | 53                    | 12.6                             |
| 1,100              | 266,700      | 252,300      | 9.0                  | 33.3                 | 51                    | 12.5                             |
| 1,150              | 237,000      | 227,000      | 9.0                  | 27.2                 | 48                    |                                  |
| 1,200              | 188,000      | 180,500      | 13.5                 | 43.2                 | 40                    | 25.3                             |

formula without causing brittleness while the product maintains ductility and good weldability. It has also been discovered that a moderate increase in the amount of molybdenum over that of my prior patents, heretofore referred to, will permit heat treatment to ultra high strength levels while tempering at a high temperature to provide less likelihood of distortion from stresses.

The alloy of this invention has the following contents in percent:

|    |               |
|----|---------------|
| C  | .40-.55.      |
| Mn | .57-.93.      |
| Si | .23-.45.      |
| Ni | .35-.70.      |
| Cr | .87-1.23.     |
| Mo | 1.88-2.27.    |
| P  | .010 maximum. |
| S  | .010 maximum. |
| V  | .49-.61.      |

Remainder iron with residual impurities.

It is important to maintain a relatively low phosphorus and sulfur content.

A desirable formula for many purposes is:

|    |                     |
|----|---------------------|
| C  | .48 approximately.  |
| Mn | .75 approximately.  |
| Si | .35 approximately.  |
| Ni | .55 approximately.  |
| Cr | 1.00 approximately. |
| Mo | 2.00 approximately. |
| P  | .010 maximum.       |
| S  | .010 maximum.       |
| V  | .50 approximately.  |

Remainder iron with incidental impurities.

The above formula may be modified by the addition of other elements and the present invention is not to be construed so as to preclude the use of small amounts of such elements as uranium 238, tungsten, columbium, or rare earth elements in the basic composition.

It is apparent from the above total that the alloy content is very low so that only a minimum of strategic

55 The short time elevated temperature properties of the alloy steel of the present invention when austenitized at 1850° F. and tempered at 1050° F. to produce the maximum strength in the secondary hardening tempering range are summarized in Table II. The test temperatures are below the corresponding temper temperature to simulate treatment necessary to be compatible with operating temperatures, i.e., the tempering temperature must be higher than the operating temperature to prevent tempering the material while in operation.

50 The elevated temperature data shows the yield and ultimate strengths to be well above 170,000 p.s.i. at 900° F. test temperature, and at 1000° F. test temperature the ultimate strength is 185,000 p.s.i. and the yield strength is 162,720 p.s.i. With these high elevated temperature properties, the present alloy is desirable for elevated temperature structural application. This data is indicative of properties obtainable when designing to operating temperature ranges.

TABLE II

Short Time Elevated Temperature Mechanical Properties  
[Heat treatment: Normalized, 1,900° F.; air quenched, 1,850° F.; tempered as shown]

| 60 | Temper Temp., ° F. | Test Temp., ° F. | Ult. Str., p.s.i. | Yield Str., p.s.i. | Elong., Percent | Red. of Area, Percent |
|----|--------------------|------------------|-------------------|--------------------|-----------------|-----------------------|
|    | 1,050              | Rm. Temp.        | 274,500           | 247,200            | 11.0            | 43.5                  |
|    | Do                 | 300              | 259,600           | 233,000            | 12.0            | 47.5                  |
|    | Do                 | 400              | 257,000           | 222,200            | 12.0            | 43.2                  |
|    | Do                 | 500              | 250,000           | 216,500            | 12.5            | 52.3                  |
|    | Do                 | 600              | 236,000           | 207,250            | 12.0            | 50.9                  |
|    | Do                 | 700              | 226,250           | 193,500            | 14.5            | 56.4                  |
|    | Do                 | 800              | 220,500           | 192,000            | 15.5            | 58.0                  |
|    | Do                 | 900              | 208,250           | 179,500            | 14.5            | 62.2                  |
|    | Do                 | 1,000            | 185,500           | 162,720            | 16.0            | 59.7                  |
| 70 | 1,100              | 1,050            | 165,260           | 141,510            | 19.0            | 64.4                  |
|    | 1,150              | 1,100            | 128,260           | 111,600            | 23.0            | 74.6                  |
|    | 1,250              | 1,200            | 58,500            | 43,300             | 54.0            | 63.6                  |

Charpy V-Notch impact properties, heat treated to 260,000 p.s.i. to 280,000 p.s.i. strength level and tested 75 at elevated temperatures are shown in Table III.

5  
TABLE III

*Elevated Temperature Impact Properties*

[Normalized, 1,900° F.; air quenched, 1,850° F.; tempered, 1,050° F.]

| Test Temp., ° F. | 1<br>Ft. Lbs. | 2<br>Ft. Lbs. | 3<br>Ft. Lbs. | Average<br>Ft. Lbs. |
|------------------|---------------|---------------|---------------|---------------------|
| 80               | 19            | 18            | 18            | 18.3                |
| 300              | 22            | 23            | 22            | 22.5                |
| 400              | 22            | 23            | 23            | 22.7                |
| 500              | 23            | 20            | 20            | 21.2                |
| 600              | 26            | 23            | 27            | 25.6                |
| 700              | 25            | 26            | 26            | 25.8                |
| 800              | 27            | 24            | 24            | 25.0                |
| 900              | 27            | 26            | 25            | 26.0                |
| 1,000            | 25            | 26            | 25            | 25.5                |

10  
TABLE IV  
*Modulus of Elasticity*

| Test Temp. (° F.) | Modulus of Elasticity (× 10 <sup>6</sup> ) |
|-------------------|--------------------------------------------|
| 80                | 30.7                                       |
| 400               | 27.4                                       |
| 500               | 26.0                                       |
| 600               | 26.7                                       |
| 700               | 27.1                                       |
| 800               | 26.5                                       |
| 900               | 24.2                                       |
| 1,000             | 24.9                                       |

6  
ELEVATED TEMPERATURE STABILITY

The elevated temperature stability of the present alloy is summarized in Table VII. The ultimate and yield strength remain unchanged, for all practical purposes, with uniform ductility, as measured by the percent elongation and reduction of area, even after 100 hours of stabilizing at 1000° F.

TABLE VII

10  
*Elevated Temperature Stability Tensile Properties*

[Heat treatment: Normalized, 1,900° F.; Air quenched, 1,850° F.; tempered at 1,050° F. Specimens held at 1,100° F. for time indicated and tested at room temperature]

| Time at 1,000° F. Hrs. | Ultimate Str., p.s.i. | Yield Str., p.s.i. | Elong., percent | Red. of Area, percent |
|------------------------|-----------------------|--------------------|-----------------|-----------------------|
| 25                     | 270,000               | 250,000            | 10.5            | 40.3                  |
| 50                     | 268,300               | 252,200            | 10.5            | 44.1                  |
| 100                    | 263,200               | 247,900            | 9.0             | 36.3                  |

15  
ROOM TEMPERATURE MECHANICAL PROPERTIES AT STRENGTH LEVELS OF 180,000-200,000 p.s.i., AND 200,000-220,000 p.s.i.

20  
25  
The data in Table VIII shows additional room temperature mechanical properties for the above two strength levels. The data further exhibits the higher strength levels obtainable with the steel of the present invention.

20  
TABLE VIII  
*Room Temperature Mechanical Properties at 200,000-220,000 p.s.i. Strength Level*

| Norm. Temp., ° F. | Quench Temp., ° F. | Temper Temp., ° F. | Ult. Str., p.s.i. | Yield Str., p.s.i. | Elong., percent | Red. of Area, percent | V-Notch Charpy Impact (Avg. 6 Tests), Ft.-Lbs. |
|-------------------|--------------------|--------------------|-------------------|--------------------|-----------------|-----------------------|------------------------------------------------|
| 1,900             | 1,850 oil          | 1,150              | 225,900           | 219,700            | 11.5            | 43.8                  | 17.0                                           |
| 1,900             | do                 | 1,175              | 215,800           | 210,000            | 12.0            | 44.9                  | 17.2                                           |
| 1,900             | 1,850 air          | 1,150              | 209,000           | 206,000            | 12.4            | 45.5                  | 21.2                                           |
| 1,900             | do                 | 1,175              | 194,700           | 193,500            | 13.5            | 48.4                  | 27.4                                           |

Angle of bend, 180° for each of the above heat treatments.

20  
TABLE V  
*Jominy End Quench Hardenability*  
[Distance from the Quenched End (Sixteenths)]

| Quench Temp. (° F.) | 1  | 2  | 3  | 4  | 5  | 6  | 8  | 10 | 12 | 14 | 16 | 20 | 24 | 28 | 32 |
|---------------------|----|----|----|----|----|----|----|----|----|----|----|----|----|----|----|
| 2,000               | 59 | 59 | 58 | 58 | 57 | 57 | 57 | 57 | 56 | 56 | 56 | 55 | 54 | 53 | 52 |
| 1,900               | 57 | 57 | 56 | 56 | 56 | 56 | 56 | 56 | 56 | 55 | 55 | 55 | 54 | 54 | 53 |
| 1,825               | 56 | 56 | 56 | 55 | 55 | 55 | 54 | 54 | 54 | 54 | 53 | 53 | 53 | 53 | 55 |

60  
CREEP RUPTURE PROPERTIES

The creep rupture properties of the improved alloy heat treated to 260,000 to 280,000 p.s.i. strength level are shown in Table VI. The properties show a very low creep rate at temperatures of 950° F. and 1000° F. This material may be used where applications of high temperature and stress are required for prolonged periods of time.

65  
TABLE VI

*Creep Rupture Properties*

[Normalized, 1,850° F.; double tempered, 1,050° F. All tests terminated after 500 hours]

| Test Temp. (° F.) | Stress, p.s.i. | Creep, percent in 50 hrs. |
|-------------------|----------------|---------------------------|
| 1,000             | 60,000         | .065                      |
| 950               | 70,000         | .0074                     |

65  
STRESS RUPTURE PROPERTIES

The stress rupture properties of the improved alloy are shown in Table IX. The properties are excellent up to 1000° F. test temperature and stresses up to 100,000 p.s.i.

70  
TABLE IX

*Stress Rupture Properties*

[Normalized, 1,700° F.; tempered, 1,050° F.]

| Test Temp., ° F. | Stress, p.s.i. | Hours to Fracture |
|------------------|----------------|-------------------|
| 1,000            | 100,000        | 98.9              |
| 1,000            | 90,000         | 148.3             |
| 1,000            | 80,000         | 270.4             |
| 1,000            | 70,000         | 465.4             |

75  
It will be understood that it is desired to comprehend within the invention and the scope of the claim thereof such equivalent materials and proportions as may be found necessary to adapt this invention to the varying conditions met in actual practice and we do not limit ourselves to these specific materials and proportions.

What I claim is:

An improved alloy steel consisting essentially of about .40-.55% carbon, about .57 to .93% manganese, about

.23-.45% silicon, about .35-.70% nickel, about .87-1.23% chromium, up to .010% phosphorus, up to about .010% sulfur, about 1.88-2.27% molybdenum in combination with about .49-.61% vanadium to produce a secondary hardening characteristic, and the remainder being iron with incidental impurities, and the metal having the ability to maintain high strength considering its low alloy content for prolonged periods of elevated temperatures with accompanying good ductility, there being an absence of temper brittleness when tempered at low tempering temperatures, said alloy steel having been heat treated by austenitizing at 1800° F.-1900° F. followed by quenching, and subsequent tempering between 1000° F. to 1100° F.

## References Cited by the Examiner

## UNITED STATES PATENTS

|             |       |          |           |
|-------------|-------|----------|-----------|
| 2,327,490   | 8/43  | Bagsar   | 75-128.85 |
| 2,919,188   | 12/59 | Furgason | 75-128.85 |
| 5 2,921,849 | 1/60  | Furgason | 75-128.85 |

## OTHER REFERENCES

Archer et al.: "Molybdenum-Steels, Irons, Alloys," Climax Molybdenum Company, New York, September 12, 1949, page 10, FIG. 7 relied upon.

DAVID L. RECK, Primary Examiner.

RAY K. WINDHAM, Examiner.